

J. SANDERS.

METHOD OF MANUFACTURING SOUND RECORD TABLETS.  
APPLICATION FILED JAN. 11, 1908.

1,192,567.

Patented July 25, 1916.



8- Basic Disk.

9- Coating of thin Solution  
or Emulsion of Record  
Material.

10- Sheet of Fibrous  
Material on  
wet Coating.

8- Basic Disk.

9- Coating of thin Solution  
or Emulsion of Record  
Material.

10- 15. 18. 21.

Coating of Solution  
or Emulsion of  
Record Material.

Fibrous Material  
Sifted on  
wet Coating.

Dipped in Fibrous  
Material while  
Coating is wet.

Powdered Record  
Material and fine  
Fibrous Material  
Mixed.

Coating of Solution  
or Emulsion of  
Record Material.

Coating of Solution  
or Emulsion of  
Record Material.

Coating of Solution  
or Emulsion of  
Record Material.

Coating of thin Sol-  
ution or Emulsion of  
Record Material.

Drying.

Drying.

Drying.

Drying.

13. 14. 16. 17. 19. 20. 23. 22.

3-



Witnessed

E. M. Edwards  
F. J. Chapman

Inventor  
Joseph Sanders.

By  
C. H. Wood

Attorneys

# UNITED STATES PATENT OFFICE.

JOSEPH SANDERS, OF WASHINGTON, DISTRICT OF COLUMBIA.

## METHOD OF MANUFACTURING SOUND-RECORD TABLETS.

1,192,567.

Specification of Letters Patent. Patented July 25, 1916.

Application filed January 11, 1908. Serial No. 410,456.

*To all whom it may concern:*

Be it known that I, JOSEPH SANDERS, a citizen of the United States, residing at Washington, District of Columbia, have invented 5 a new and useful Method of Manufacturing Sound-Record Tablets, of which the following is a specification.

This invention has reference to improvements in the method of manufacturing 10 sound record tablets, the term tablets being used in this connection to include either a tablet before the sound record groove is impressed therein or the finished tablet with the groove impressed therein.

15 The sound record tablet hereinafter described is not herein claimed since it forms the subject matter of and is claimed in another application filed by me on April 29, 1908, under Serial No. 429,931, for sound 20 record tablets, as a division of this application.

At the present time the principal type of sound record tablets is the disk shaped tablets, and these are commonly made of a mixture 25 of shellac and other materials, including fibrous material, usually cotton fiber cut into short lengths and known as cotton flock. The usual practice of making sound record tablets is to take a mixture of such materials 30 with the ingredients already incorporated, and soften the same by heat and then impress a sound record groove from a matrix of the same into the heated and thereby softened material, the heat and pressure being 35 sufficient to produce a faithful copy of the matrix into the heated material which is pressed out into the form of a disk of appropriate size and is allowed to cool and set under pressure. Such sound record tablets

40 with the sound groove impressed therein have become known, commonly, as sound records and are also known by various trade names, but for reasons which need not be here stated, I prefer to designate the type 45 of record tablets described as a gramophone sound record, and the material as gramophone record material. Among other gramophone record materials that described in Letters Patent No. 787,001, granted to me

50 on April 11, 1905, under the title of "Composition of matter for sound record tablets," is particularly adapted for use in the present invention. Furthermore the type of tablet described in Letters Patent No. 956,904, for sound record tablets, granted to me on May 3, 1910, is a type of tablet to

which the present invention is particularly applicable. However the surfacing material applied in the manner described in said Letters Patent last named is not perfectly adapted to all conditions.

The ordinary gramophone sound record groove is about 1/250 of an inch, more or less, in width, and of commensurate depth, being sometimes as shallow as 1/500 of an inch and at other times deeper in accordance with the desires of the recording expert. Some experts use very deep and wide grooves compared with those used by others. The standard pitch of the spiral on which the groove is produced is approximately one hundred turns to the inch. The result is that while a comparatively narrow, shallow groove has at all times comparatively wide plateaus between the turns even when the turns are closest due to the sinuosities of the groove representing sound waves, a deep and wide groove will at times produce narrow plateaus between closely approaching turns and oftentimes the walls of a groove are quite thin for a considerable distance into the face of the tablet.

A shellac containing gramophone record material where the shellac is associated with oxid of iron or some other like material is quite brittle when flock is omitted for reasons which will hereinafter appear and the thin walls between two turns of deep grooves are unable to resist the lateral thrust or strain due to the guiding of the stylus and the parts controlled thereby and these walls often break down under such thrust or strain, the walls where merging into the plateaus being shattered or chipped away and the record becomes defective for reproduction to a commensurate extent.

It is one of the objects of the present invention to overcome this defect without sacrificing any of the advantages inherent in a record disk comprising a basic structure of material other than that used for the record receiving surface and this object is realized by incorporating in the surfacing of record material a suitable quantity of fibrous material which will serve to very markedly 100 chipping or shattering or breaking down of the walls of the groove in the manner and under the conditions stated.

In the aforesaid Patent No. 956,904, the surfacing material is applied in liquid form, 110 that is the shellac is dissolved and the other materials are held in suspension in the solu-

tion, but the presence of fibrous material renders it difficult to produce an even coating, even though the fibrous material be cut very fine, the fiber absorbing much of the 5 solvent. It is therefore not an uncommon practice in making up tablets in the manner set forth in the said Letters Patent to omit the flock from the surface layer. Furthermore when the surface layer is deposited 10 from an emulsion and this layer is made fairly heavy the quick exterior drying of the material retards the drying out of the remainder for a comparatively long time, or several thin coats must be applied to get the 15 requisite thickness of the surfacing.

The production of a surface coating of the desired record material of the requisite thickness but which shall be quick drying and which can be applied without additional 20 handling constitutes another part of the present invention and consists in applying to the matrix structure a cementing material to which the final coating in powdered form is applied, the solvent of the material, when 25 such solvent is employed quickly evaporating because of the large exposed surface.

The usual method of manufacturing the record material by softening the shellac and then mixing therewith the other ingredients 30 does not cause the infiltration of the fibers of the fibrous material by the shellac. Therefore the material is more or less hygroscopic and many such records become defective in damp climates, particularly in 35 warm moist climates.

To obviate this defect constitutes a still further object of the present invention and this is done by applying an additional coating of a thin solution or emulsion of the 40 record material from which flock has been omitted. By this means the fibrous material of the record surface has its fibers encapsulated in the non-fibrous record material and they are thereby either so infiltrated 45 with the record material or so protected thereby as to be unaffected by moisture even when subjected to the effects of moist torrid climates such as are sometimes encountered in the tropics.

50 The invention will be best understood from a consideration of the following detail description taken in connection with the accompanying drawings forming a part of this specification, in which drawings,—

55 Figure 1 is a partially schematic section of a small portion of a sound record of the gramophone or disk type, showing the comparatively shallow form of record groove. Fig. 2 is a similar view showing the deeper 60 and wider form of record groove. Fig. 3 is a schematic sectional view of a tablet made in accordance with the present invention and illustrating one phase of the process of manufacture. Fig. 4 is a similar view to 65 Fig. 3 to illustrate a more advanced step

in the manufacture. Fig. 5 is a schematic sectional view of a portion of a record tablet made in accordance with the present invention and indicating a sound record impressed therein. Fig. 6 is a diagram indicating consecutive steps in the manufacture of a sound record in accordance with the present invention, and Fig. 7 is a like diagram showing some variations of the steps in the manufacture from that shown in Fig. 6.

Referring to Figs. 1 and 2, there is shown a base 1 and a surfacing 2. The proportions of these two parts are of course greatly exaggerated since the entire tablet need not exceed about one-eighth of an inch in thickness and the surfacing material may be one one-hundredth of an inch or less in thickness, and under some circumstances may be considerably less than one one-hundredth of an inch in thickness. The basic material is 85 preferably, though not necessarily, made of cardboard or pasteboard or other cheap fibrous material which, for reasons which need not be entered into here, but which are fully disclosed in my aforesaid application, 90 is sized with rosin or other like material, but preferably a material which will soften under heat and which is hard and firm when cold. Nor is it necessary for the purposes of the present invention that the base or under- 95 structure be made of a single disk, as for instance, a disk of cardboard made of macerated fibrous material, but may be made up of a number of sheets of fibrous material as is present in laminated cardboard, or the 100 base may be made of a disk of cardboard preferably suitably sized upon which is secured a thin disk of paper carrying the record material. This last-named structure and its purposes and advantages are set 105 forth in my application #239,961, filed January 6, 1905, for gramaphone record tablets. It need only be stated here that the inter- 110 posed sheet of paper between the record-receiving material and the base facilitates the manufacture and also aids in preventing any admixture of materials used in the base with the record-receiving material where the materials contained in the base or some of them are detrimental to the said record-receiving 115 material. This extra sheet of paper is indicated by the reference numeral 3 in Fig. 5.

In Fig. 1 there are shown two adjacent grooves 4, 4, and these may be taken as indicative of the more shallow type of gramophone or disk record grooves where the normal separation of the turns of the spiral constituting the record groove is approximately one one-hundredth of an inch, while the width of the grooves themselves is considerably less, say, approximately one two-hundred and fiftieth of an inch, and the depth, say, one five-hundredth of an inch more or less. These figures are of course to be taken only as approximate. In such com- 120 125 130

paratively narrow and shallow grooves the intervening plateau 5 is of considerable width and the thickness of material between adjacent spirals of the groove is well able 5 to withstand the side thrust of a reproducing stylus when being actuated by the record groove and constrained to follow the sinuosities representing sound waves, even when the sinuosities of one member of the spiral 10 groove are in the opposite sense to the sinuosities of the next adjacent member of the spiral groove, as will sometimes happen, for even then the plateau is of considerable width and the walls of the groove approach 15 the same at such an obtuse angle that the intervening record material between two even closely approaching adjacent members of the groove is still of such thickness as to well withstand the thrust of the stylus. 20 However, it is the custom of some recording experts to form the record grooves much deeper and wider than those indicated in Fig. 1, and such deep wide record grooves are indicated at 6, 6, in Fig. 2. With such 25 grooves the plateaus are normally narrower than the normal plateau of the tablet of Fig. 1, and when the sinuosities of the adjacent spiral members are in opposite sense, as they often are, so that a particular portion of the 30 groove in one spiral member is brought into very close relation to a particular portion of the groove of the other spiral member, then the intervening plateau is reduced to very narrow limits and the steepness of the 35 walls of the groove leave much less record material between the two adjacent positions of the spiral members of the groove than under the conditions of Fig. 1. The result is that a brittle record material without the 40 presence of flock or other strengthening fiber, is unable to withstand the thrust of the reproducing stylus and pieces of the intervening record material between the walls of the adjacent portions of the grooves are 45 shattered and broken away, as roughly indicated at 7 in Fig. 2, thus marring the reproducing qualities of the record tablet and sometimes destroying its usefulness for further reproduction. 50 Gramophone or disk record materials made of shellac and other ingredients are too brittle to be rolled out into very thin sheets for application to the fibrous or other base, and consequently can only be economically 55 applied to such base either in the manner hereinafter described or when the shellac is dissolved in a suitable solvent, and the other materials are held in suspension in the shellac solution so as to form what may 60 be termed an emulsion of the gramophone or disk record material. Such emulsion is readily applied by a brush or by dipping the basic disk or paper vehicle therein. However, the presence of flock renders it 65 very difficult to produce from an emulsion

an even layer with the materials properly distributed and a surface coating so formed is comparatively slow drying because, among other reasons, the flock absorbs a material portion of the solvent, as before stated. So 70 where the shallow grooves are used the surface layer of record material is made of shellac and oxid of iron or some similar material without the admixture of flock.

The flock, which term may be taken as 75 descriptive of any suitable fibrous material in a suitably finely cut state is added to the surface material composed of shellac and other ingredients, while it is in the form of a thin solution or emulsion which is coated 80 upon the basic disk or upon the paper vehicle by means of a brush or by dipping or in any other suitable manner, thus producing a thin coating of the record material.

In Figs. 6 and 7 there is displayed schematically the several steps in the production of a record tablet blank in accordance with the present invention, and in this schematic representation the first step in the process is the preparation of the basic disk 90 which may, for the purposes of the invention, be considered as either a disk 1 of cardboard or pasteboard or similar material which preferably is impregnated with a sizing such as rosin or other material capable 95 of softening when heated and which is hard and resisting when in a cold state. This sizing may or may not extend entirely through the disk but should extend to a sufficient distance into the disk from the 100 surface thereof to maintain the fibers of the disk when they are compacted under the pressure necessary for the impress of the sound record groove, in such compressed state, by cementing such fibers together and 105 preventing them from again expanding to their original condition when the pressure is relieved, thus preventing distortions and irregularities or other defects from being 110 formed in the record-receiving surface.

In Figs. 6 and 7, such basic disk, whether 115 formed of a suitably sized cardboard disk or a cardboard disk with a paper facing, or however formed, is indicated by the rectangle 8, and following this is another rectangle 9 which represents the step of coating the basic disk with a thin solution or emulsion of the record material, or as will hereinafter appear in connection with the method of constructing the tablet blank displayed in Fig. 6, this second step may consist in the application of shellac alone or some other like material.

Referring now to Fig. 7 only, in conjunction with Figs. 3 and 4, the rectangle 10 indicates a step which may follow the coating of the disk with the thin solution or emulsion of record material. According to one method of procedure, a thin sheet of fibrous material, such for instance, as cotton bat- 130

ting, may be laid upon the wet coating formed of a thin solution of record material. In Fig. 3, the coating formed of the thin solution of record material is indicated at 11, while the fibrous material thereupon is indicated at 12. The sheet of fibrous material will take up the greater portion of the wet coating by absorption, and if the coating of record material be thick enough 15 then the fibrous material will become entirely embedded therein and when dry may be heated and impressed with a sound record matrix. But because of the slowness of drying thick coatings of the solution or 20 emulsion of record material, the first coating may be thin, and in order to obtain the necessary body of record material there may be an additional coating of a solution or emulsion of record material, as indicated 25 by the rectangle 13, and following this the disk may be dried, which last step is indicated by the rectangle 14.

Instead of using a sheet of fibrous material the latter may be cut up into very 25 short lengths and then deposited on the wet coating, and this step is indicated by the rectangle 15. After this there may be another coating of a solution or emulsion of record material, as indicated by the rectangle 30 16, and may be followed by drying, as indicated by the rectangle 17. Or instead of depositing the fibrous material on the wet coating, the basic disk, after being coated with a thin solution or emulsion of record 35 material, may be dipped into a mass of finely cut fibrous material, which step is indicated by the rectangle 18, and this may afterward receive an additional coating of a solution or emulsion of record material, as indicated by 40 the rectangle 19 to be followed by the drying indicated by the rectangle 20. In the first of the ways of applying the fibrous material described with reference to the representation of Fig. 7, the sheet of fibrous material will adhere to the wet coating and the amount of fibrous material is determined 45 solely by the thickness of such sheet. In the case of depositing fine fibrous material on the wet coating there may be more deposited than is needed, and the surplus may be jarred off since enough of the fibrous material will adhere to the wet coating for the purposes of the invention. In the case of dipping the coated disk into a mass of 55 the fibrous material, the latter will adhere in sufficient quantities to the surface of the disk and what fails to adhere will gravitate off the disk or may be jarred off.

In whatever manner the fibrous material 60 is caused to adhere to the surface of the disk with its initial coating of a solution or emulsion of record material, and when the second coating of the emulsion or solution of record material is applied then there is upon the 65 disk a coating of record material composed

of shellac and oxid of iron, if that be the particular material used, with an imprisoned mass of fibrous material, which latter is present in sufficient quantity to impart the requisite strength and resistance to the shattering action of the reproducing stylus when the deep and wide record grooves like those shown at 6 in Fig. 2 are impressed into the record surface.

In Fig. 6, there is displayed another 75 method of producing the record surface upon a basic disk of a material not well adapted for the reproductions of sound from a groove impressed by a sound record matrix, which record surface may receive 80 the deep and wide groove of Fig. 2, and then successfully resist the action of the reproducing stylus of the gramophone type of reproducing machine. In the process as displayed in Fig. 6, the basic disk is the same 85 as before and is preferably made of cardboard or pasteboard, or some such material, with a sizing of rosin or other suitable material for the purpose, and with or without the interposed sheet 3 of paper. Upon this 90 disk is produced a coating of a thin solution or emulsion of record material or this may even, under some circumstances, be a thin coating of shellac only, or in case the binding element of the record material be some 95 other substance than shellac then the initial coating may or may not contain shellac, depending upon the binding element of the record material used.

In the method displayed in Fig. 6, the 100 third step represented by the rectangle 21 differs somewhat from the corresponding steps in the methods represented in Fig. 7. For this third step the record material is composed of shellac, oxid of iron or other 105 similar and suitable material; and fibrous material provided in a powdered state of sufficient fineness for the purpose, and the basic disk with its coating of a thin solution or emulsion of record or other material, 110 while still wet is dipped in or has deposited upon it the powdered record material, which gives it all the elements of record material used for solid disks and may be termed complete record material.

Assuming that the coating of the thin solution or emulsion of record or other material first placed upon the disk is of sufficient body, then the requisite quantity of the powdered complete record material will adhere 120 and the surplus may be allowed to gravitate or be jarred off, and the disk so coated may be allowed to dry. When such a disk is afterward heated to the requisite degree to soften the record material and the tablet is 125 subjected to the pressure of the matrix, then the surfacing of record material is pressed into conformity with the matrix surface and will be found of sufficient thickness and durability to successfully resist the action of 130

the point of the stylus of the reproducing machine the same as though a sufficiently thick coating of the record material had been originally produced upon the surface 5 of the disk directly from a solution or emulsion of the record material. But a decided advantage arises from the production of the record-receiving surface in the manner just described, for the reason that the record 10 material is composed of a binding material such as shellac, a hardening material such as oxid of iron or similar substance, and a strengthening material such as flock or other fibrous substance, thus permitting the 15 production in such surface of a sound record groove of comparatively great width and depth with the separating walls so strong as to resist the action of a pointed stylus, even though these walls be comparatively thin. 20 Furthermore, the production of a surface suitable for receiving the record impressions directly from a solution or emulsion of the record material aside from the difficulty of so producing a record surface containing 25 flock or other such strengthening element, is necessarily a slow process, since, if a sufficiently thick coating be initially produced then the surface evaporation of the solvent forms a skin layer which retards the drying 30 of the deeper portions of the coating for a comparatively long time. Or, if this be avoided by using several thin coatings to build up a coating of sufficient thickness, then there is the attendant multiplicity of 35 handling and the time taken in drying, which adds very materially to the expense of producing these tablets.

By the use of a thin initial coating and then applying the fibrous material thereto, 40 or by applying the complete record material to this thin coating while the said record material is in a powdered state, the drying is greatly facilitated because of the absorption in the fibrous material or into the 45 powdered record material of the initial coating, whereby the exposed surface of the latter to the evaporation of the solvent is greatly enlarged and the drying proceeds at a very rapid rate. Moreover, but a small 50 amount of solvent is necessary, and any deleterious effects of the solvent on the shellac is thereby minimized or entirely avoided.

In the process indicated in Fig. 6 another step may follow the application of the powdered complete record material, and this consists in the application of another coating of a thin solution or emulsion of record material indicated by the rectangle 22 to be followed by the drying of the tablet indicated by the rectangle 23.

In all the processes of forming the record tablet the final coating may be of a thin solution or emulsion of the record material without the fibrous material, or in the particular instance set forth, this coating con-

sists of a thin solution or emulsion of shellac with oxid of iron or other suitable hardening material.

The purpose of the second coating is to thoroughly encapsule or imprison the particles of the fibrous material, for such material is more or less hygroscopic, and when subjected to moisture, especially in damp climates, and more particularly in moist tropical climates, the fibrous material, unless 70 protected against the moisture, is liable to absorb sufficient moisture to spoil the finished record tablet for the reproduction of sound, when the sound groove is impressed therein, because of the presence of the contained moisture, which softens the surface of the tablet so that it is no longer resistant to the point of the stylus to the extent necessary for tablets of this character.

In Fig. 5 is shown a portion of a record 80 disk constructed in accordance with the present invention, but with the proportions greatly exaggerated. In this figure the record grooves are indicated at 24, while the record receiving material is indicated at 25 90 very much thicker than the paper layer 3, but this is done only for clearness of illustration, while in practice this layer 25 need not be thicker than one one-hundredth of an inch and may actually be considerably 95 thinner.

The sizing in the basic disk 1 is indicated in the several figures by shading 26 which is not intended to illustrate the actual conditions present in the disk but simply to indicate the infiltration of the sizing into the disk, it being understood that the sizing may extend entirely through the disk or may be denser at the surface than within the disk or may under some circumstances extend but 100 partially through the disk, it only being necessary that the fibers of the disk be sufficiently anchored by the sizing to prevent the swell of the disk after having once been subjected to the pressure used for producing 110 the sound grooves in the surfacing of record-receiving material. The sizing also prevents absorption of the record-receiving material into the understructure.

To give a specific example, the present invention may be successfully carried out by the use of a pasteboard or cardboard disk of suitable thickness with a suitable sizing such as rosin, and upon this sized base the coating of a thin solution or emulsion of 115 shellac and oxid of iron may be produced either directly or upon a paper disk, which in turn is applied to the sized cardboard disk. Then upon this coating while the latter is still wet, there may be produced another coating made up of a powdery mixture of shellac, oxid of iron and flock, say cotton flock, in proper proportions such as set forth in my Letters-Patent #787,001, before referred to, and sufficient of this record ma- 125 130

terial will adhere to the wet coating to produce the coating needed for the reception of the record groove. Finally, over this adherent coating of the complete record material another coating made up of a solution or emulsion of shellac and oxid of iron may be applied and the article be then dried, after which the tablet may be heated and the record groove impressed from a matrix in the usual manner.

The present invention may also be successfully carried out by the use of a fibrous understructure of suitable thickness to which the cementing layer may be applied in such manner as to infiltrate the understructure to an extent sufficient for the purposes of the invention, that is, when the tablet is subjected to heat and pressure the cementing material infiltrating the understructure will 20 constitute a sizing which will soften under such heat, and when hardened will cement the fibers of the understructure together so that the latter will not swell after the pressure is relieved. The cementing material 25 which may, for instance, be a shellac solution or a solution of a material which does not deteriorate the material of the record-receiving surface may be allowed to dry and may be then made adhesive by heat, and the powdered record-receiving material may then be applied to such adhesive surface. When the tablet again becomes cold the powdered material will adhere strongly to the cementing material and the tablet may again 30 be subjected to heat and be subjected to the impress of the matrix in the usual manner. It is possible to use for the cementing and sizing material cheap grades of commercial shellac which are more or less adulterated 35 with resinous substances, and this cementing material will not interfere to any marked extent with the record-receiving qualities of the surfacing material.

When a sizing suitable for cementing the 45 surface material is used it may be employed in the form of a solution and be either brushed upon the fibrous base, or the latter may be dipped into the solution for a length of time determined by the depth it is desired 50 that the sizing shall sink into the fibrous base.

When a paper sheet is interposed between the main portion of the fibrous base and the surfacing material, then the shellac solution 55 may be used to infiltrate the paper sheet and act as a sizing therefor as well as a cement for the powdered record-receiving material.

The invention may also be successfully 60 carried out by the application of powdered record material composed of a binder such as shellac and a hardening material such as oxid of iron or other similar material without the admixture of flock, and this record-receiving material may be deposited upon

the cementing surface or the tablet may be dipped into a mass of the powdered material either while the surface of the tablet is still wet to a greater or less degree with the solvent or when the cementing material has 70 been permitted to dry and become hard and is then heated and softened to make it adhesive to the powdered material.

When the paper sheet is used, the base or understructure may consist of some cheap 75 thermo-plastic material not suited for the record-receiving surface. Such material may be made up of rosin or other such material, as a binder and baryta, infusorial earth, or other like hardening material, while flock 80 or other fibrous material may or may not be added, as desired.

From the foregoing description of the several ways of carrying out the invention it will be seen that the application of fibrous 85 material to a suitable base in order to make a tablet having a record receiving surface coating of fiber-containing record material produced thereupon, may be performed by causing an adhesive condition of the surface 90 of the tablet in any of the ways described, and then applying the fibrous material in a dry state to such adhesive surface whether the fibrous material be applied uncoated with other materials or whether it be an element of a composition suited for the record receiving coating of the tablet, such composition being, when applied, in a dry, powdered state.

It is not to be presumed that I am by any 100 means limited to the several materials mentioned, for any ingredients which will answer the requirements incident to the manufacture of gramophone or disk record tablets may be used, nor am I limited in the use 105 of hardening or both hardening and binding materials for sound record receiving surfaces, to shellac as the binder for the other elements of the record receiving material, for other resinous substances and some gums 110 may be used for the purpose.

My invention also includes any material suitable for gramophone or disk tablet record receiving surfaces wherein the addition of cotton flock or other suitable substances 115 is advantageous in imparting strength and reducing the brittleness or frangibility of such record receiving surfaces under the conditions of use.

What is claimed is:—

1. The method of manufacturing sound record tablets with a record-receiving surface coating of suitable fiber-containing record material, which consists in first causing 125 an adhesive condition of the surface to be coated, then applying fibrous material in a dry state to such surface while the latter is in the adhesive condition, then permitting the surface coated to become solid or hard and anchor the powdered material thereto, 130

- then heating the tablet to soften the record-receiving material, and impressing a sound-record matrix therein.
2. The method of manufacturing sound record tablets with a record-receiving surface coating of suitable fiber-containing record material, consisting in first applying a solution or emulsion of suitable record receiving material free from fiber containing record material, and then applying fibrous material to the same before the solvent has evaporated.
3. In the production of sound record tablets, first providing a suitable tablet base or understructure, then applying thereto a coating of a solution or emulsion of suitable record material free from fibrous material, and then applying to the said coating suitable record material containing fibrous material, said fiber-containing record material being in dry powdered form and applied before the solvent of the first named coating has evaporated.
4. The method of producing sound record tablet blanks consisting in first coating the basic portion of the tablet with an adhesive and then applying powdered record material containing fibrous material to said adhesive while the latter is in condition to bind the powdered material to the base.
5. The method of producing sound record tablets consisting of coating the basic portion of the tablet with a thin solution or emulsion of record material, then while the first coating is still wet applying fibrous material and then applying another coating composed of a thin solution or emulsion of record material.
6. The method of producing a sound record tablet blank consisting in coating a fibrous base with a thin solution or emulsion of an adhesive suitable for use in gramophone or disk record tablets and then applying fibrous record-material in a loose state to such coating while the latter is in a condition to cement the applied fibrous material to the fibrous base.
7. The method of producing sound record tablet blanks consisting in coating a fibrous base with a thin solution or emulsion of non-fibrous record material and then applying to said coating before the solvent has evaporated a powdered record-receiving material containing fibrous material.
8. The method of producing sound record tablet blanks consisting in coating a fibrous base with a thin solution or emulsion of non-fibrous record material and then applying to said coating before the solvent has evaporated a powdered record-receiving material containing fibrous material, and then applying another coating of a thin solution or emulsion of a non-fibrous record-receiving material.
9. The method of producing sound record tablet blanks consisting in producing upon a sized disk of fibrous material, a coating of a thin solution or emulsion of non-fibrous record-receiving material, and then applying to the said coating a powdered record material containing fibrous material, before the solvent of the initial coating has evaporated.
10. The method of producing sound record tablet blanks consisting in producing upon a sized disk of fibrous material a coating of a thin solution or emulsion of non-fibrous record-receiving material, then applying to the said coating the powdered record material containing fibrous material before the solvent of the initial coating has evaporated, and then applying another coating of a thin solution or emulsion of the non-fibrous record material.
11. The method of producing sound record tablets consisting in first producing a basic member of fibrous material sized with material capable of softening when heated, then coating the basic body with a thin solution or emulsion of non-fibrous record material also capable of softening under heat, and then producing upon the said coating before the solvent of the latter has evaporated, another coating of powdered record material containing fibrous material, said last-named record material being capable of softening under heat.
12. The method of producing sound record tablet blanks consisting in forming a base of fibrous material infiltrated with rosin, producing thereupon a coating of a thin solution or emulsion of non-fibrous record-receiving material, capable, when dry, of softening under heat, producing upon said coating while still containing solvent, a coating formed of powdered record material containing fibrous material, said last-named record material being thermo-plastic and finally producing upon the coating of powdered record material another coating of a thin solution or emulsion of the record material like that of the first-named coating.
13. The method of producing sound record tablets consisting in first producing a basic disk of fibrous material containing rosin, producing thereupon a coating from a thin solution or emulsion of a record-receiving material capable when dry of softening under heat, applying to said coating while still containing solvent, a layer of fibrous thermo-plastic record-receiving material, then producing upon a second layer a third layer composed of a thin solution or emulsion of record-receiving material like the first-named layer, then drying the tablet blank so formed and then heating the tablet blank to soften the thermo-plastic material carried thereby, and finally impressing a sound record matrix into the heated and thereby softened record surface.

14. In the manufacture of gramophone record tablets, first producing a thermoplastic fibrous base, then causing an adhesive condition of the surface of the base, then producing thereupon a coating of suitable fiber-containing thermoplastic record material applied in a dry powdered condition to said surface while still in an adhesive condition, then permitting the surface of the base 16 to return to the non-adherent condition, and anchor the powdered record material thereto, then rendering the coating plastic by heat, and impressing a sound record matrix therein.
15. 16. The method of manufacturing gramophone sound record tablets with a surface coating of a suitable fiber-containing record material, consisting in first producing a thermoplastic fibrous base, then applying 20 thereto an adhesive in solution, then applying fibrous material to the adhesive before the solvent has evaporated, and then, after the adhesive has become dry, softening the record receiving surface by heat and impressing a sound record groove therein from a matrix thereof.
17. 18. The method of manufacturing gramophone sound record tablets with a surface coating of a suitable fiber-containing record material, consisting in first producing a thermoplastic fibrous base, then applying thereto a solution of record material free from fibrous material, then applying dry, powdered, fiber-containing record material, and then, after the coating has become dry, 35 softening the record receiving surface by heat and impressing a sound record groove therein from a matrix thereof.

In testimony that I claim the foregoing as my own, I have hereto affixed my signature 40 in the presence of two witnesses.

JOSEPH SANDERS.

Witnesses:

ISAAC W. NORDLINGER,  
J. THOMAS SOTHORON.